

Nov. 15, 1949

H. MORROGH

2,488,511

NODULAR CAST IRONS AND THE MANUFACTURE THEREOF

Filed Jan. 25, 1949

8 Sheets-Sheet 1



Fig.1—Typical example of "graphite-flake aggregate" nodule in malleable cast iron having sulphur present as manganese sulphide. Etched in 5 per cent nital.  $\times 300$ .



Fig.2—Spherulitic nodule in malleable iron having sulphur present as FeS. Etched in picric acid.  $\times 350$ .



Fig.3—General structure of untreated remelted pig iron, 1.2-in. test bar. Etched in picric acid.  $\times 100$ .



Fig.4—Microstructure of cerium-treated remelted pig iron, 1.2-in. test bar. Etched in picric acid.  $\times 100$ .



Fig.5—Duplex structure of hyper-eutectic spherulite present in cerium-treated iron. Unetched.  $\times 1500$ .

INVENTOR  
**HENTON MORROGH**  
By *Raymond L. Clegg*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 2



Fig. 6—Typical segregation of hypereutectic spherulites at inner surface of centrifugally cast cylinder liner (cerium-treated iron). Etched in picric acid.  $\times 100$ .



Fig. 7—Centrifugally cast liner. Structure at a point distant from inner surface. All graphite is in form of quasi-flakes. Etched in picric acid.  $\times 100$ .



Fig. 8—Untreated remelted hematite pig iron cast in 3-in. diameter bar. Etched in picric acid.  $\times 60$ .



Fig. 9—Remelted pig iron with 0.040 per cent Ce, cast in 3-in. diameter bar. Picric acid etch.  $\times 60$ .



Fig. 10—Remelted hematite with 0.101 per cent Ce, cast in 3-in. diameter bar. Picric acid etch.  $\times 60$ .

INVENTOR  
**HENTON MORROGH**  
BY  
*Roy J. Steenland*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 3



Fig.11—General structure of 1.2-in. bar with Ce addition (No.1, Table 3). Etched in picric acid.  $\times 100$ .



Fig.12—Microstructure of typical 1.2-in. bar with cerium and ferro-silicon addition (No.2, Table 3). Picric acid etch.  $\times 100$ . Note many spherulitic nodules.



Fig.13—Structure of 1.2-in. bar with cerium and ferro-silicon addition (No.3, Table 3) is almost entirely spherulitic. Etched in picric acid.  $\times 100$ .



Fig.14—Photomicrograph of 1.2-in. bar with cerium and ferro-silicon addition (No.4, Table 3) shows small amount of quasi-flake graphite. Picric acid etch.  $\times 100$ .



Fig.15—Metal treated simultaneously with misch metal and silicon-manganese-zirconium shows spherulitic nodules with only a trace of quasi-flake graphite in pearlite and ferrite matrix. Etched in picric acid.  $\times 100$ .

INVENTOR

**HENTON MORROGH**

By

*Roy G. Tamm*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 4



Fig. 16—White iron structure at apex of chill wedge made from metal treated with cerium alone shows only a trace of hyper-eutectic graphite. Picric acid etch.  $\times 60$ .



Fig. 17—Structure of chill wedge,  $\frac{3}{8}$ -in. from apex, treated with cerium alone, shows rather more graphite but still is predominantly white. Picric acid etch.  $\times 60$ .



Fig. 18—Apex of chill wedge, cast from double-treated metal, shows only a very small amount of carbide in the structure. Etched in picric acid.  $\times 60$ .



Fig. 19—Chill wedge structure,  $\frac{1}{8}$ -in. from apex, cast from double-treated metal, shows presence of only small amount of free cementite. Picric etch.  $\times 60$

INVENTOR  
**HENTON MORROGH**

By

*Roy A. Stearns*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 5



Fig. 20—Structure of 1.2-in. bar (No. 1, Table 4) with 0.016 per cent Ce, produced by double treatment process. Some quasi-flake graphite. Picric acid etch.  $\times 100$ .



Fig. 21—Wholly spherulitic structure of 1.2-in. bar (No. 2, Table 4) with 0.031 per cent Ce, produced by double treatment process. Etched in picric acid.  $\times 100$ .



Fig. 22—Microstructure of 0.6-in. bar (No. 1, Table 4) with 0.016 per cent Ce, double treatment process, shows some quasi-flake graphite. Picric acid etch.  $\times 100$ .



Fig. 23—Structure of 0.6-in. bar (No. 2, Table 4) with 0.031 per cent Ce, produced by double treatment process, shown to be wholly spherulitic. Picric acid etch.  $\times 100$ .

INVENTOR

**HENTON MORROGH**

BY

*Raymond*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 6



Fig. 24—Structure of 1.6-in. bar (Table 5) in copper-containing double-treated iron, shows spherulitic nodules in matrix of pearlite. Etched in picric acid.  $\times 100$ .



Fig. 25—Spherulitic nodule at high magnification in 0.6-in. bar (Table 5) in copper-containing double-treated iron. Note radial structure. Picric etch  $\times 1250$ .



Fig. 26—Photomicrograph showing duplex structure of nodule in 1.6-in. bar (Table 5) in copper-containing double-treated iron. Etched in picric acid.  $\times 500$ .



Fig. 27—Microstructure of nodular iron with 4.13 per cent silicon content. Etched in picric acid.  $\times 100$ .

INVENTOR

HENTON MORROGH

By

*Raymond*  
R. ATTORNEY

Nov. 15, 1949

H. MORROGH

2,488,511

NODULAR CAST IRONS AND THE MANUFACTURE THEREOF

Filed Jan. 25, 1949

8 Sheets-Sheet 7



Fig. 28—Photomicrograph showing structure of 1.2-in. bar (Table 6) in single treatment nodular iron with 0.50 per cent phosphorus. Picric acid etch.  $\times 100$ .



Fig. 29—Microstructure of 1.2-in. bar (No. 2, Table 7) produced in double-treated nodular iron with 2.92 per cent Mn content. Etched in picric acid.  $\times 100$ .



Fig. 30—Structure of 0.875-in. bar in untreated nickel-containing iron (Table 9). Picric acid etch.  $\times 100$ .

INVENTOR

**HENTON MORROGH**

By

*Roy K. Leonard*  
his ATTORNEY

Nov. 15, 1949

H. MORROGH

2,488,511

NODULAR CAST IRONS AND THE MANUFACTURE THEREOF

Filed Jan. 25, 1949

8 Sheets-Sheet 8



Fig. 31—Microstructure of 0.875-in. bar in nodular nickel-containing iron (Table 9). Picric etch.  $\times 100$ .



Fig. 32—Microstructure of 1.2-in. bar (Table 11) in cupola-melted double-treated iron, shows spherulitic nodular graphite. Etched in picric acid.  $\times 60$ .

INVENTOR  
**HENTON MORROGH**  
By  
*Roy F. Leonard*  
his ATTORNEY

## UNITED STATES PATENT OFFICE

2,488,511

## NODULAR CAST IRON AND THE MANUFACTURE THEREOF

Henton Morrogh, Handsworth, England, assignor to British Cast Iron Research Association, Alvechurch, Birmingham, England

Application January 25, 1949, Serial No. 72,575

19 Claims. (Cl. 75—123)

1

This invention relates to nodular cast irons and the manufacture thereof. More particularly, the invention relates to the manufacture of gray cast irons of novel type which contain a variable small proportion of cerium uncombined with sulphur and in which part or all of the graphitic carbon content is in the form of nodules visible under the microscope, which irons have not been subjected to a heat-treatment process for the purpose of producing that graphite structure but, on the contrary, possess their characteristic structure in the as-cast state, and are further characterized by markedly improved mechanical properties as compared with previously known gray cast irons having generally similar analyses, respectively, but not containing cerium.

Ordinary gray cast irons have their graphitic carbon distributed throughout the metallic matrix in the form of flakes, the size and shape of which vary considerably according to composition, cooling rate, method of melting, ladle treatment, etc. These graphite flakes interrupt the continuity of the metallic matrix and so render the material brittle and non-ductile.

For many years, skilled workers in the metallurgy of cast iron have endeavored to improve the mechanical properties of gray cast iron as regards strength and resistance to shock without at the same time rendering it so hard as largely to lose the advantage of good machinability normally characterizing gray cast iron. The past two decades, especially, have witnessed the gradual evolution of high-duty gray cast iron, particularly in the field of castings for the engineering and automobile industries. This evolution began with the realization of the importance of the control of carbon and silicon and the relative adjustment of these two elements in cast iron. This phase was accompanied by the development and application of the hot-mold process and the utilization of high-steel mixtures in cupola practice.

Next, the inoculation technique was introduced and developed to a process of indispensable com-

2

mercial utility. The aim of this technique has been to give random flake structures in irons of relatively low carbon and silicon contents and to inhibit and control the chilling tendencies of such irons. All of these developments have been accompanied by advances in the use of special alloying elements, such as chromium, nickel, copper, molybdenum, etc., to strengthen the metallic matrix of cast iron.

10 These advances have culminated in the production of the nickel-molybdenum acicular cast irons which, in commercial production, represent a combination of most of the earlier developments—acicular irons are essentially irons with controlled low carbon contents; they are usually inoculated and have a combination of alloying elements which, after an appropriate heat-treatment, confer the maximum strengthening effect on the metallic matrix. However, one frequent 15 objection to present high-duty gray cast irons, particularly when alloyed with molybdenum, is their poor machinability.

In striking contrast to all gray cast irons previously known, those of the present invention 20 are always characterized and distinguishable by the fact that at least a substantial part of their graphitic carbon content exists in nodular form with resultant notable improvement in mechanical properties of the material. It has long been 25 recognized that the mechanical properties of gray cast iron could be considerably improved if the graphite could be obtained in the nodular instead of flake form. Prior to the present invention, however, no way by which to produce 30 gray cast iron having a nodular graphite structure has ever been devised, and the objective 35 appeared to be unattainable. It was known, of course, that by producing castings of white iron, and then subjecting the white iron castings to a prolonged annealing treatment, the white cast iron would be converted into malleable cast iron having a nodular graphite structure; but malleable cast iron is a product quite different in 40 various respects from gray cast iron, with which

the present invention exclusively is concerned, and is readily distinguishable therefrom.

It has now been found that the problem of producing gray cast iron having, in the as-cast state, a nodular graphitic structure and, thereby, improved mechanical properties, can be solved by treating the gray iron melt to be cast with a material, specifically cerium, which will function in the melt both as a desulphurizer and also as a carbide stabilizer.

The process of the present invention involves, in its simplest form, only the addition of an appropriate amount of cerium to a molten cast iron of appropriate composition, and solution of cerium in the iron, shortly before casting.

The principal composition requirements for the production of nodular irons by this process are:

1. The iron to be treated must solidify gray in the untreated condition; the process is not applicable to a white iron. With this reservation, the matrix structure may be pearlitic, ferritic, a mixture of ferrite and pearlite, martensitic, acicular, or austenitic.

2. In irons to be treated which contain less than 10 per cent of nickel (nickel need not be present), a high carbon content is necessary and the iron should be hypereutectic, that is, it should have a carbon content in excess of that given by the formula:  $4.3 - \frac{1}{3}$  (per cent Si + per cent P).

3. Silicon content can have any value, but should most desirably be within the range of 2.3 to 7 per cent. With the special-purpose irons containing 10 to 15 per cent silicon, only the hypereutectic graphite can be obtained with certainty in the nodular form.

4. Any deficiency of silicon may be compensated for by the presence of nickel and/or copper in appropriate amounts. In this respect 3 per cent of nickel and/or copper is to be considered equivalent to 1 per cent of silicon. Alternatively, a deficiency of silicon may be compensated for by the addition of ferrosilicon or similar material to the molten metal.

5. The sulphur content of the molten metal to which the cerium addition is to be made should be low, preferably not more than 0.03 per cent or thereabouts, and it is generally not commercially practicable to treat directly, without preliminary desulphurization, an iron whose sulphur content exceeds 0.06 per cent. One of the functions of the cerium addition is to reduce the sulphur content of the treated metal to a value not exceeding about 0.02 per cent as a maximum and most desirably to below 0.015 per cent, and even as low as 0.005 per cent.

6. The phosphorus content should not exceed about 0.6 per cent, and should preferably be less than 0.1 per cent.

7. Manganese, copper, nickel, chromium and molybdenum may be present in any amounts, singly or in any combination, provided the other conditions listed above are observed.

8. After treatment with cerium, the solidified castings must contain at least a certain minimum amount (0.015 to 0.02 per cent) of the element dissolved in the metallic matrix. However, the amount of cerium dissolved in the matrix must not be so large as to give white cast iron.

Of the foregoing requirements, the most important from the standpoint of practically successful use of the process are those covering the carbon and sulphur contents.

Investigations and discussions concerning the influence of cerium in cast iron appear in the literature, but an examination of this literature

shows that previous investigators failed to obtain nodular structures because they added too much and obtained white-iron structures, or the irons were white before treatment, or the sulphur contents of the irons being treated were too high, or the irons were not hypereutectic, or the cerium yield (amount available for solution as such in the metallic matrix) was poor due to the method of making the addition, several of these factors being combined in some instances. No previous investigators have claimed that nodular structures were or could be produced in cast irons by the addition of cerium.

As a result of long and difficult investigation leading to the present invention, it has become apparent that the first major effect of cerium when added to molten cast iron is to combine with the sulphur to form a cerium-sulphur compound which floats to the surface of the metal. This accounts for the desulphurizing effect of the element. So long as the sulphur content of the metal is above about 0.015 per cent, or above 0.02 per cent at the most, only this desulphurizing action will take place. Cerium is not free to dissolve in or alloy with the molten iron until the sulphur content has reached this low value. The higher the sulphur content of the metal, the larger is the amount of cerium required to achieve desulphurization, and hence to obtain a given amount of cerium (not combined with sulphur) dissolved in the metal.

After the sulphur content has been reduced to a value of 0.02 per cent, or at any rate to a value of about 0.015 per cent, metallic cerium enters into solution in the molten cast iron, and this cerium, when present in amounts greater than about 0.02 per cent, functions as a powerful carbide stabilizer. It is this dissolved cerium in excess of 0.02 per cent which is the operative factor in the process for the production of nodular graphite structures in the as-cast state.

Notwithstanding the distinct novelty of the cast irons of the present invention, it should be clearly understood that nodular graphite structures are by no means unknown, in and of themselves. As has already been pointed out hereinabove, their production in iron castings by heat-treatment has long formed the basis of the process for the production of malleable cast iron. For commercial malleable cast iron, the material is cast in the form of hard and brittle white cast iron which contains no graphitic carbon. These white iron castings are then annealed at elevated temperatures, and during this treatment the hard and brittle iron carbide in the white iron decomposes to give graphitic carbon, commonly termed temper carbon, which exists in roughly spheroidal aggregates or nodules. These temper carbon nodules, by virtue of their approximately spheroidal shape, do not interrupt the continuity of the metallic matrix to the same extent as does flake graphite and so, if the total carbon content is sufficiently low, a material of relatively good shock-resistance and ductility may be obtained.

Hitherto this thermal treatment of a solid white cast iron has been the only known way of producing nodular graphite. The present invention obviates the necessity for the lengthy high-temperature annealing treatment of the malleable iron process. However, it should not be misunderstood that the production of nodular gray cast irons by the present novel process in any way constitutes a means of producing malleable cast iron by a short cut; for the mechanical properties of the as-cast nodular gray cast irons, as

well as other characteristics, are quite different from those of malleable cast irons as will more fully hereinafter appear. It will accordingly be seen that nodular gray cast iron is a new ferrous material, having properties by which it is differentiated and readily distinguished from ordinary gray cast iron on the one hand, and from malleable cast iron on the other, but having some of the characteristics of each.

In further explaining the nature and underlying principles of the invention, reference will be made to the accompanying drawings, Figures 1 to 32 inclusive, which are reproductions of photomicrographs of cross sections of various metal specimens, a number of which are typical of the novel gray cast irons of the invention.

Before giving further details of the present invention, it may be well to point out that the nodular temper-carbon structure found in malleable cast iron and produced by annealing white iron castings can occur in either of two forms according to the composition of the white iron being annealed. When the white iron has all its sulphur predominantly in the form of manganese sulphide, each nodule in the resulting malleable iron consists of an apparently random clump or aggregate of small graphite flakes, the degree of dispersion of which may vary between wide limits. A typical example of this structure, which may be conveniently termed a "graphite-flake-aggregate" nodule, is shown in Fig. 1.

However, where the manganese content of the malleable cast iron is inadequate to balance the sulphur, so that iron sulphide occurs in the material, the temper carbon has a spherulitic structure, a typical example of which is illustrated in Fig. 2. Since spherulitic nodules are obtained also in the nodular gray cast irons of the present invention, it is of some interest and importance to understand and appreciate this graphite structure.

At this point, it should be stated that these structures can be observed only in microspecimens in which the graphite itself is polished. A method for accomplishing this has been described by the present applicant in The Journal of The Iron and Steel Institute, vol. 143 (1941), pages 195-205.

Nodules of graphite having this spherulitic structure each consist of an aggregate of graphite crystallites radiating from a common center or nucleus. The closely packed basal planes of these crystallites are, in general, oriented at right angles to the radii of the spheroid. Graphite spherulites tend to be more perfectly spheroidal

Resuming detailed discussion of the invention, it may be pointed out that when cerium is added to hypereutectic cast irons, and when the final sulphur content is below about 0.015 per cent and the cerium content of the treated metal is above about 0.02 per cent, all the hypereutectic graphite is obtained as well-formed spherulites in the resultant casting. When the silicon content of such an iron is sufficiently high to prevent formation of the white iron eutectic, there is also obtained another form of graphite which originates from the eutectic complex and which, although it sometimes resembles normal flake graphite in general appearance, especially when the cerium percentage is near the minimum, nevertheless differs radically therefrom. For convenience, this sometimes flakelike graphite is herein termed "quasi-flake graphite." Its manner of formation is quite different from that of normal flake graphite and so, also, is its effect upon the characteristics of the resultant gray cast iron. Indeed, as will more fully be pointed out hereinafter, its effect upon said characteristics is such and, with increasing amounts of cerium it becomes so increasingly nodular in appearance, that the term "nodular," as herein employed, is to be understood as including within its scope such quasi-flake graphite as may frequently occur in gray cast irons produced in accordance with the principles of the invention.

The following example illustrates this effect of cerium on hypereutectic cast irons.

#### EXAMPLE 1

A 50 lb. charge of hematite pig iron having the following percentage analysis:

|              |       |
|--------------|-------|
| Total carbon | 3.98  |
| Silicon      | 3.19  |
| Manganese    | 0.78  |
| 40 Sulphur   | 0.028 |
| Phosphorus   | 0.040 |

was melted in a crucible furnace and cast, at a temperature of 1380° C., into test bars of four different sizes.\* A further similar melt was carried out, but in this case a 28-gram addition of pure cerium was added to the molten metal before casting. Mechanical properties and chemical analyses of the two sets of bars are shown in Table 1.

\* The transverse, deflection and tensile figures given in this application disclosure for 2.1, 1.6, 1.2, 0.875 and 0.6-in. diameter bars were obtained on bars cast and tested according to British Standard Specification 786/1938; the impact figures were obtained on bars tested according to British Standard Specification 1349/1947; the 3-in. diameter bars were tested in transverse on 18-in. centers.

Table 1.—Mechanical properties of untreated<sup>1</sup> and cerium-treated<sup>2</sup> cast irons

| Test Bar Diameter, in. | Transverse Rupture Stress, p. s. i. |         | Deflection, in. |         | Tensile Strength, p. s. i. |         | BHN    |         | Impact Strength, ft.-lb. |         | Compression Strength, p. s. i. |         | Shear Strength, p. s. i. |         |
|------------------------|-------------------------------------|---------|-----------------|---------|----------------------------|---------|--------|---------|--------------------------|---------|--------------------------------|---------|--------------------------|---------|
|                        | W/O Ce                              | With Ce | W/O Ce          | With Ce | W/O Ce                     | With Ce | W/O Ce | With Ce | W/O Ce                   | With Ce | W/O Ce                         | With Ce | W/O Ce                   | With Ce |
| 1.6                    | 51,500                              | 99,000  | 0.20            | 0.32    | 25,100                     | 55,050  | 154    | 186     | ---                      | ---     | 71,600                         | 127,100 | ---                      | ---     |
| 1.2                    | 64,500                              | 101,500 | 0.28            | 0.38    | 32,050                     | 55,500  | 160    | 198     | 12                       | 43      | ---                            | ---     | 36,500                   | 49,700  |
| 0.875                  | 68,870                              | 105,400 | 0.18            | 0.23    | 37,200                     | 59,550  | 162    | 199     | ---                      | ---     | ---                            | ---     | ---                      | ---     |
| 0.6                    | 68,900                              | 128,500 | 0.11            | 0.22    | 41,650                     | 69,020  | 198    | 239     | ---                      | ---     | 118,750                        | 153,000 | ---                      | ---     |

<sup>1</sup> Analysis of remelted pig iron: total carbon 3.77; silicon, 3.05; manganese, 0.73; sulphur, 0.022; phosphorus, 0.039 per cent.

<sup>2</sup> Remelted pig iron with cerium additions: total carbon, 3.72; silicon, 3.13; manganese, 0.74; sulphur, 0.007; phosphorus, 0.038; cerium, 0.040 per cent.

in shape than the flake-aggregate nodules, and application of the term "spherulite" or "spherulitic" is confined herein to aggregates having a radial fiber structure such as that illustrated in Fig. 2.

Microstructures of all the untreated bars show mixtures of undercooled and normal flake graphite in matrices of ferrite with some pearlite—the amount of flake graphite increasing and the amount of pearlite decreasing with increasing

section size. The microstructure of the untreated 1.2-in. bar is shown in Fig. 3. The treated bars all showed hypereutectic spherulites, together with quasi-flake graphite in a matrix of ferrite with some pearlite. The structure of the treated 1.2-in. bar is shown in Fig. 4.

The structure shown in Fig. 4 is, judged by previous standards, completely novel and, bearing in mind the distribution of the graphite, it is easily understandable that the mechanical properties of the treated material are at a distinctly higher level than those of the untreated material. It is to be observed in Table 1 that, even with this simple cerium addition to a high carbon and relatively high silicon iron, a material is obtained which immediately falls into the category of a high-duty cast iron.

Although it is to be understood that the invention is not dependent upon any theory of operation, the available evidence indicates that the mechanism of solidification of the type of structure illustrated in Fig. 4 is probably about as is assumed in the following suggested explanation.

The hypereutectic spherulitic nodules form in the melt before solidification of the metallic phases begins. It is not known for certain whether these graphite spherulites are deposited directly from the melt or whether they form by the decomposition of a carbide phase. While the possibility of the latter has to be considered, it is not easy to imagine and it involves a case of extremely rapid carbide decomposition.

The remainder of the melt solidifies as a "eutectic" or, more correctly, a binary complex of austenite and cementite which decomposes shortly after solidification to give the quasi-flake graphite. The presence of the hypereutectic spherulites appears to initiate the rapid decomposition of the "eutectic" cementite after solidification of the iron.

It will be observed in Fig. 4 that the hypereutectic nodules are surrounded in each case by a volume of metal entirely free from the quasi-flake graphite. The reason for this becomes apparent when these nodules are examined at a high magnification, when each is found to have, in addition to the characteristic radial spherulitic structure, a duplex structure consisting of a central spherulite of nodular graphite surrounded by a peripheral layer of graphite.

Such a duplex structure is seen in Fig. 5, which shows a hypereutectic spherulite in a cerium-treated iron at a fairly high magnification. This micrograph has been taken under plane polarized light. The central core of this duplex nodule represents the actual hypereutectic graphite, and the peripheral layer represents the graphite arising from the decomposition of the surrounding "eutectic" cementite which has crystallized onto the hypereutectic spherulite. This explains the absence of quasi-flake graphite in the vicinity of each nodule in Fig. 4.

Each hypereutectic nodule appears to have a "sphere of influence" within which all further graphite is made to crystallize on the existing hypereutectic nucleus. This provides a clue leading to a refinement of the simple method of cerium addition to the melt, whereby a larger proportion, or even the whole, of the graphite can be obtained in the spherulitic nodular form. This further refinement or more complete and optimum embodiment of the invention will be herein-after described in detail but, from what has already been said, it will be seen that if the number of hypereutectic spherulites in a given volume of

metal could be so increased that all their "spheres of influence" overlapped, then all of the graphite should occur in the form of duplex spherulitic nodules with a further improvement in mechanical properties. A preliminary indication of the validity of this latter idea is found by studying the structures of centrifugally cast cerium-treated cast irons.

When cerium-treated hypereutectic cast irons are centrifugally cast, the hypereutectic spherulites forming in the liquid are forced to points most distant from the mold face, by virtue of their low relative density. In the centrifugal casting of cylinder liners, for instance, a segregation of these nodules is obtained along the inner surface of the casting. By this segregation the number of hypereutectic nodules is thus artificially increased so that their "spheres of influence" overlap.

Figure 6 shows a typical segregation of these hypereutectic spherulites near the inner surface of a centrifugally cast cylinder liner made in a cerium-treated hypereutectic cast iron. It will be seen that no quasi-flake graphite occurs in the vicinity of this segregation. At points nearer the mold face containing very few hypereutectic nodules, all of the graphite was in the form of quasi-flakes, as illustrated in Fig. 7.

These two micrographs clearly indicate that entirely spherulitic nodular graphite structures can be achieved by increasing the number of hypereutectic spherulites. This ideal structure of spherulitic nodular graphite has been obtained by the use of what will be referred to later as the "double-treatment process."

In the example already given the cerium was added to the molten cast iron in the form of the pure element. In this form cerium is a very expensive addition, but it can be added in a variety of cheaper forms, among which misch metal ("mischmetal") is perhaps the most convenient. Misch metal usually contains between 43 and 50 per cent cerium, together with the other rare earths and a little iron and manganese. The presence of these other elements does not influence the efficacy of cerium in producing nodular structures in cast irons, and for this purpose they can be ignored.

Misch metal, in pieces of appropriate size, dissolves readily in cast irons at all temperatures above 1200° C. Its solution in cast iron is not explosive or violent in any way. Misch metal has been used as a cerium addition in all the remaining examples to be given hereinafter. However, the addition can be made, if desired, in any other suitable form such as cerium carbide, for example, or as any of the various available alloys of cerium, among which may be mentioned ferrocerium, copper-cerium, nickel-cerium, silicon-cerium, etc.

Cerium not combined with sulphur in cast iron is a powerful carbide stabilizer, and so, for any given section size, there is an upper limit of cerium which must not be exceeded if white iron structures are to be avoided. This remark applies only to the cerium content as found by analysis of the solidified casting when the sulphur content is not in excess of about 0.015 per cent. Because of the carbide stabilizing influence of cerium its effect can best be studied in relatively large sections.

#### EXAMPLE 2

To illustrate the effect of increasing additions of cerium, 270 lb. of pig iron of the following

composition was melted in an oil-fired crucible furnace:

|              |       |
|--------------|-------|
| Total carbon | 3.79  |
| Silicon      | 2.80  |
| Manganese    | 0.53  |
| Sulphur      | 0.028 |
| Phosphorus   | 0.015 |

Five test bars, each of 21-in. length and 3-in. diameter, were cast in green sand molds. For this, five lots of metal each weighing 50 lb. were taken from the furnace. No addition was made to the metal in the first ladle, but increasing amounts of misch metal were added to the metal in the remaining four ladles. The actual additions were: Tap 1—no addition; Tap 2—50 grams misch metal; Tap 3—65 grams misch metal; Tap 4—90 grams misch metal; Tap 5—100 grams misch metal. The mechanical properties and cerium analyses of these bars are given in Table 2.

Table 2.—Mechanical properties and cerium analyses

| Bar No. | Transverse Rupture Stress, <sup>1</sup> p. s. i. | Deflection, <sup>1</sup> in. | Tensile Strength, p. s. i. | BHN | Ce, per cent |
|---------|--------------------------------------------------|------------------------------|----------------------------|-----|--------------|
| 1       | 30,470                                           | 0.21                         | 15,000                     | 98  | Nil          |
| 2       | 85,090                                           | 0.21                         | 40,100                     | 167 | 0.040        |
| 3       | 101,100                                          | 0.35                         | 50,200                     | 176 | 0.053        |
| 4       | 106,600                                          | 0.34                         | 53,800                     | 181 | 0.072        |
| 5       | 115,600                                          | 0.42                         | 58,850                     | 179 | 0.101        |

<sup>1</sup> Tested on 18-in. centers.

Transverse rupture stress, deflection and tensile strength show a progressive improvement with increasing cerium content. The microstructures of these bars also showed a progressive change with increasing cerium content. The untreated bar No. 1 had coarse flake graphite in a matrix of ferrite with some pearlite, as is shown in Fig. 8; bar No. 2 had a few hypereutectic spherulites with quasi-flake graphite, as illus-

large sections. For thin sections, alternative methods must be applied to obtain an entirely nodular structure. It has been pointed out hereinabove that, if the number of hypereutectic nuclei could be increased sufficiently, all of the graphite would occur in spherulitic nodular form and the quasi-flake graphite would be absent.

Production of this ideal structure can be realized in practice through addition of a graphitizing inoculant simultaneously with, or preferably after, the cerium addition. This treatment of the molten metal will be referred to as the "double treatment" process. Suitable graphitizing inoculants have been found to be 80 per cent ferro-silicon, silicon-manganese-zirconium, and calcium silicide, the best response having been obtained with the first and second. It is important that the inoculant be not added before the cerium addition as the success of the operation depends upon obtaining the solution of the cerium before the inoculant.

Owing to the extremely rapid rate of solution of misch metal in cast iron, this condition may be achieved even when the inoculant and misch metal are added simultaneously. For the inoculant to have the required effect it is necessary to add sufficient, in the case of silicon-manganese-zirconium or ferro-silicon, to give a definite increase in silicon of not less than about 0.2 per cent, but no useful purpose is served by using amounts giving silicon yields in excess of 0.5 per cent.

Results given in Table 3 illustrate the effect of adding varying amounts of 80 per cent ferro-silicon for the same addition of misch metal in each case. These figures are average values, obtained from four 1.2-in. bars cast in each case from 50 lb. of metal treated as follows: Tap 1—70 grams misch metal; Tap 2—70 grams misch metal + 2 oz. 80 per cent ferro-silicon; Tap 3—70 grams misch metal + 4 oz. 80 per cent ferro-silicon; Tap 4—70 grams misch metal + 8 oz. 80 per cent ferro-silicon.

Table 3.—Effect of 80 per cent ferro-silicon additions

| Tap No. | Composition, per cent |      |      |       |       |       | Transverse Rupture Stress, p. s. i. | Deflec-tion, in. | Tensile Strength, p. s. i. | BHN | Impact, ft.-lb. |
|---------|-----------------------|------|------|-------|-------|-------|-------------------------------------|------------------|----------------------------|-----|-----------------|
|         | T. C.                 | Si   | Mn   | S     | P     | Ce    |                                     |                  |                            |     |                 |
| 1       | 3.67                  | 2.67 | 0.86 | 0.005 | 0.051 | 0.010 | 127,200                             | 0.60             | 58,200                     | 221 | 54              |
| 2       | 3.52                  | 2.73 | —    | —     | —     | 0.051 | 138,000                             | 0.60             | 71,000                     | 233 | 91              |
| 3       | 3.49                  | 2.89 | —    | —     | —     | 0.058 | 138,900                             | 0.60             | 74,900                     | 238 | 84              |
| 4       | 3.50                  | 3.03 | —    | —     | —     | 0.061 | 142,000                             | 0.77             | 75,700                     | 231 | 70              |

trated in Fig. 9; with increasing amounts of cerium in bars Nos. 3, 4 and 5 the quasi-flake graphite became more nodular in appearance until bar No. 5 had the structure shown in Fig. 10.

That quasi-flake graphite differs from normal flake graphite is made clear when Figs. 8 and 9 are compared, and when the enormous difference in mechanical properties between bars Nos. 1 and 2 is considered. The relative amounts of ferrite and pearlite did not change appreciably with increasing cerium content, but in spite of this there was a sharp increase in hardness when the structure changed from the normal to the quasi-flake graphite.

#### Double-treatment technique

The influence of relatively large amounts of cerium in causing the aggregation of the quasi-flake graphite can be utilized only in relatively

large sections. Transverse rupture stress, tensile strength and impact strength show a marked increase with the first addition of inoculant (compare bars 1 and 2). The impact results are particularly striking—these figures are obtained on a 0.798-in. diameter unnotched test piece which rarely gives a value in excess of 30 ft.-lb. for high-duty gray cast iron, and only occasionally a value as high as 50 ft.-lb. for acicular cast iron.

Microstructures of typical bars from these four taps are shown in Figs. 11, 12, 13 and 14. The bar from tap 1 (Fig. 11) is seen to have partially aggregated quasi-flake graphite; the bar from tap 2 (Fig. 12) has many spherulitic nodules with only a little quasi-flake graphite; the bar from tap 3 (Fig. 13) has an almost entirely spherulitic structure; the bar from tap 4 (Fig. 14) has only a little quasi-flake graphite. The matrix structure does not differ greatly through this series.

11  
EXAMPLE 3

Similar results can be obtained when the metal is treated simultaneously with the cerium addition and the inoculant, as is shown by the following example. A mixture of 70 grams of misch metal and 6 oz. of silicon-manganese-zirconium was placed in the bottom of a ladle and 60 lb. of metal run onto it. Four bottom-run 1.2-in. bars were cast and their average mechanical properties and the analysis of one bar are:

## Chemical analysis, per cent—

|              |       |
|--------------|-------|
| Total carbon | 3.71  |
| Silicon      | 2.96  |
| Manganese    | 0.54  |
| Sulphur      | 0.010 |
| Phosphorus   | 0.033 |
| Cerium       | 0.051 |

## Mechanical properties—

|                                     |         |
|-------------------------------------|---------|
| Transverse rupture stress, p. s. i. | 140,900 |
| Deflection, in.                     | 0.60    |
| Tensile, strength, p. s. i.         | 72,100  |
| Brinell hardness number             | 241     |
| Impact strength, ft.-lb.            | 71      |

The microstructure of one of these bars is shown in Fig. 15, and is seen to have spherulitic nodules with only a trace of quasi-flake graphite in a matrix of pearlite and ferrite.

Application of the double treatment process tends to offset the carbide stabilizing influence of the cerium and hence to reduce the danger of chilling. This effect automatically permits the use of higher percentages of cerium in the solidified casting, a factor which in addition helps to improve the structure of the material.

## EXAMPLE 4

To illustrate the reduction in chilling tendency with the double treatment technique, the following example may be cited. A wedge test piece having the dimensions of one inch at base, 2 in. from apex to base, and 6 in. long was cast in a dry sand mold. The wedge was fractured transversely and gave a chilled zone approximately  $\frac{3}{4}$ -in. deep. The percentage analysis of this wedge was:

|              |       |
|--------------|-------|
| Total carbon | 3.77  |
| Silicon      | 2.69  |
| Manganese    | 0.56  |
| Sulphur      | 0.011 |
| Phosphorus   | 0.024 |
| Cerium       | 0.061 |

In this case no double treatment was applied, and the white iron structure of the apex of the wedge is shown in Fig. 16. Only a trace of hypereutectic graphite can be seen. The structure  $\frac{3}{4}$ -in. from the apex is shown in Fig. 17 and, while rather more graphite can be seen, the structure still is predominantly white.

On the other hand, when a similar wedge of the composition

|              |       |
|--------------|-------|
| Total carbon | 3.70  |
| Silicon      | 2.73  |
| Manganese    | 0.59  |
| Sulphur      | 0.008 |
| Phosphorus   | 0.055 |
| Cerium       | 0.061 |

was cast after the application of the double treatment process, it showed no visible chill when fractured. The structure of the apex of this wedge is shown in Fig. 18, where only a very small amount of carbide can be seen. At a point  $\frac{3}{4}$ -in.

from the apex only traces of free cementite exist, as is shown in Fig. 19.

It appears that an optimum amount of cerium is necessary, even with the double treatment technique, to cause the structure to be entirely spherulitic. When the cerium content is below this value quasi-flake graphite may persist in the structure. This is shown by the results given in Table 4, and the structures shown in Figs. 20, 21, 22 and 23.

Table 4.—Analyses and mechanical properties—cerium and silicon-manganese-zirconium additions

|         |                            | Composition, per cent                    |                              |                          |                          |                                      |       |
|---------|----------------------------|------------------------------------------|------------------------------|--------------------------|--------------------------|--------------------------------------|-------|
|         |                            | T. C.                                    | Si                           | Mn                       | S                        | P                                    | Ce    |
| Set 1   |                            | 3.90                                     | 2.96                         | 0.31                     | 0.006                    | 0.024                                | 0.016 |
| Set 2   |                            | 3.90                                     | 3.10                         | 0.52                     | 0.007                    | 0.023                                | 0.031 |
| Set No. | Bar Size, in.              | Transverse Rupture Stress, p. s. i.      | Deflection, in.              | BHN                      | Impact Strength, ft.-lb. | Tensile Strength, p. s. i.           |       |
| 1       | 1.6<br>1.2<br>0.875<br>0.6 | 104,500<br>114,100<br>122,900<br>142,000 | 0.51<br>0.68<br>0.39<br>0.35 | 179<br>189<br>213<br>239 | 32<br>46<br>76<br>—      | 54,800<br>62,700<br>65,100<br>75,900 |       |
| 2       | 1.6<br>1.2<br>0.875<br>0.6 | 133,900<br>143,000<br>153,900<br>164,000 | 0.90<br>1.02<br>0.66<br>0.43 | 190<br>199<br>231<br>252 | 89<br>—<br>—<br>—        | 73,500<br>73,900<br>77,300<br>88,100 |       |

<sup>1</sup> Full capacity of the Izod impact machine used is 120 lb.

Table 4 gives the analyses and mechanical properties of two sets of test bars prepared by treating two 50-lb. taps of metal poured from the same melt with the following additions: Set 1—40 grams misch metal followed by 5 oz. silicon-manganese-zirconium; Set 2—60 grams misch metal followed by 5 oz. silicon-manganese-zirconium.

Microstructures of the 1.2-in. bars are shown in Figs. 20 and 21, and those of the 0.6-in. bars in Figs. 22 and 23. The 1.2-in. and 0.6-in. diameter bars of set 1 clearly have some quasi-flake graphite, whereas this form of graphite is entirely absent and the structure is wholly spherulitic in the bars from set 2.

## EXAMPLE 5

With silicon contents below about 2.3 per cent and in the absence of other graphitizing elements, the chilling tendency of cerium-treated nodular irons, even when the double treatment process is applied, is so great that very careful control is necessary in order to avoid chilling in sections of less than  $\frac{3}{4}$ -in.

However, when any deficiency of silicon is compensated for by the presence of appropriate amounts of copper and/or nickel a material of very good mechanical properties can be obtained, even in relatively thin sections. An example of this type is illustrated by the results given in Table 5, which are taken from a double treated nodular iron of the following percentage composition:

|              |       |
|--------------|-------|
| Total carbon | 3.80  |
| Silicon      | 2.17  |
| Manganese    | 0.92  |
| Sulphur      | 0.015 |
| Phosphorus   | 0.052 |
| Cerium       | 0.054 |
| Copper       | 2.17  |

Table 5.—Mechanical properties of double treated nodular iron

| Bar Size, in. | Transverse Rupture Stress, p. s. i. | Deflection, in. | Tensile Strength, p. s. i. | BHN | Impact Strength, ft.-lb. |
|---------------|-------------------------------------|-----------------|----------------------------|-----|--------------------------|
| 1.6           | 150,000                             | 0.30            | 89,000                     | 260 | 88                       |
| 1.2           | 157,000                             | 0.40            | 79,200                     | 288 | 92                       |
| 0.875         | 181,000                             | 0.30            | 96,500                     | 302 | 94                       |
| 0.6           | 206,500                             | 0.27            | 114,000                    | 333 | —                        |

The general structure of the 1.6-in. bar from this set is shown in Fig. 24 to consist of spherulitic nodules associated with ferrite in a matrix of pearlite. Figure 25 shows a spherulitic nodule in the 0.6-in. bar at a high magnification—the radial structure can be clearly seen. Occasionally in such samples the duplex structure of the nodules is revealed in a quite interesting manner. A typical instance of this is shown in Fig. 26, which shows a duplex nodule in the 1.6-in. bar. The central hypereutectic nucleus can be clearly seen with the remainder of the graphite, still in the spherulitic form, attached to the nucleus at only a few points.

#### EXAMPLE 6

The double treatment can be applied and useful mechanical properties obtained with silicon contents as high as 6 per cent. With increasing silicon up to about 5 per cent the transverse rupture strength, tensile strength and Brinell hardness number do not change appreciably, but the shock-resistance drops progressively. The following figures, obtained on a fairly high silicon iron, illustrate the type of results which can be obtained:

#### Chemical analysis, per cent

|              |       |
|--------------|-------|
| Total carbon | 3.14  |
| Silicon      | 4.13  |
| Manganese    | 0.85  |
| Sulphur      | 0.004 |
| Phosphorus   | 0.046 |
| Cerium       | 0.051 |

#### Mechanical properties (1.2-in. diameter bar)—

|                                     |         |
|-------------------------------------|---------|
| Transverse rupture stress, p. s. i. | 141,500 |
| Deflection, in.                     | 0.38    |
| Tensile strength, p. s. i.          | 77,500  |
| Brinell hardness                    | 234     |
| Impact strength, ft.-lb.            | 29      |

The microstructure of this sample consisted of spherulitic nodules in a matrix of ferrite with a little pearlite, as is shown in the photomicrograph of Fig. 27 at a magnification of 100.

#### EXAMPLE 7

The use of cerium for the production of nodular cast irons cannot be extended to phosphorus contents in excess of about 0.6 per cent because this element appears to lower the solubility of cerium in the melt. At relatively high temperatures (in excess of 1450° C.) the cerium dissolves readily, but on cooling it is deposited from the melt at a temperature of about 1380° C. in the form of a cerium-rich alloy.

For instance, 50 lb. of a phosphoric pig iron was melted in a crucible furnace and treated with 100 grams of misch metal when at a temperature of 1470° C. The addition appeared to dissolve readily, but as the metal cooled prior to pouring a thick scum developed on the surface of the metal. This was skimmed off and the rest of the metal poured into test bars. The

scum and the test bars gave the following figures on subsequent analysis:

| 5            | Composition, per cent |              |
|--------------|-----------------------|--------------|
|              | Scum                  | Metal Poured |
| Total Carbon | 3.33                  | 3.46         |
| Silicon      | 2.37                  | 2.61         |
| Manganese    | 0.72                  | 0.84         |
| Sulphur      | 0.076                 | 0.036        |
| Phosphorus   | 1.20                  | 1.44         |
| Cerium       | 4.80                  | Not detected |

Obviously, there is a considerable segregation of cerium and sulphur in the material skimmed from the surface of the liquid metal.

Although nodular structures can be obtained with up to 0.6 per cent phosphorus, the mechanical properties fall off progressively with increasing amounts of this element. The results shown in Table 6 give the mechanical properties of a fairly high phosphorus iron of the following percentage composition:

|    |              |       |
|----|--------------|-------|
| 25 | Total carbon | 3.60  |
| 25 | Silicon      | 2.67  |
| 25 | Manganese    | 0.54  |
| 25 | Sulphur      | 0.007 |
| 25 | Phosphorus   | 0.50  |
| 25 | Cerium       | 0.031 |

#### Table 6.—Mechanical properties of 0.50 per cent phosphorus iron

| 35 | Bar Size, in. | Transverse Rupture Stress, p. s. i. | Deflection, in. | Tensile Strength, p. s. i. | BHN | Impact Strength, ft.-lb. |
|----|---------------|-------------------------------------|-----------------|----------------------------|-----|--------------------------|
|    | 1.6           | 82,500                              | 0.20            | 43,400                     | 241 | —                        |
| 40 | 1.2           | 81,800                              | 0.20            | 45,300                     | 242 | —                        |
| 40 | 0.875         | 94,100                              | 0.14            | 43,900                     | 256 | 11                       |
| 40 | 0.6           | 81,300                              | 0.09            | 40,300                     | 255 | —                        |

This metal was treated with misch metal alone—the double treatment was not applied. The results obtained may therefore be compared with those in Table 1. The microstructure of the 1.2-in. bar from this series had large hypereutectic spherulites and quasi-flake graphite in a matrix of pearlite with phosphide eutectic. This structure is shown in Fig. 28.

#### EXAMPLE 8

Provided that the iron will solidify gray before treatment the manganese content of a nodular cast iron may have any value. The general effect of increasing amounts of manganese is to inhibit the formation of ferrite, even with fairly high silicon contents, and ultimately to give entirely pearlitic structures and, if sufficient of the element is present, to give martensitic structures. The results given in Table 7 show the tensile strength and hardness of two relatively high manganese nodular irons produced by the double treatment process. These high manganese irons were cast in the form of 1.2-in. diameter bars.

#### Table 7.—High manganese nodular irons

| 70 | No. | Composition per cent |      |      |       |       |       | Tensile Strength, p. s. i. | BHN |
|----|-----|----------------------|------|------|-------|-------|-------|----------------------------|-----|
|    |     | T. C.                | Si   | Mn   | S     | P     | Ce    |                            |     |
| 70 | 1   | 3.63                 | 2.91 | 2.01 | 0.009 | 0.044 | 0.067 | 72,800                     | 256 |
| 70 | 2   | 3.61                 | 3.00 | 2.92 | 0.017 | 0.034 | 0.057 | 81,100                     | 319 |

Bar No. 1, containing 2.01 per cent manganese, had a microstructure consisting of uniformly dis-

diluted spherulitic nodules in a matrix of about 70 per cent pearlite and 30 per cent ferrite. The graphite structure of bar No. 2 was very similar to that of bar No. 1, but the matrix in this case was almost entirely pearlitic with a small amount of martensite and a little carbide. The structure of bar No. 2 is illustrated in Fig. 29. The tensile strength and hardness values of the irons are seen to increase as the structure becomes pearlitic.

#### EXAMPLE 9

High manganese nickel-containing austenitic irons may be treated with cerium to give nodular structures with a considerable improvement in mechanical properties. This is illustrated by the results given in Table 8, which show the mechanical properties of an untreated and a cerium-treated nickel-manganese austenitic iron. The double treatment was not applied in this case. The untreated material had a structure of coarse flake graphite in a matrix of austenite, and the treated material had a nodular structure in a similar matrix with a little carbide.

Table 8.—Nickel-manganese austenitic iron

| Bar Size, in. | Transverse Rupture Stress, p. s. i. | Deflection, in. | Tensile Strength, p. s. i. | BHN  | Impact Strength, ft.-lb. |
|---------------|-------------------------------------|-----------------|----------------------------|------|--------------------------|
| 1.6           | 32,300                              | 0.60            | 11,960                     | 86.8 | -----                    |
| 1.2           | 37,000                              | 0.80            | 13,210                     | 90.7 | -----                    |
| 0.875         | 37,600                              | 0.38            | 15,000                     | 102  | 105                      |
| 0.6           | 42,100                              | 0.32            | 16,350                     | 102  | -----                    |

Untreated: T. C., 3.28; Si, 3.08; Mn, 5.8; S, 0.022; P, 0.072; Ni, 11.87 per cent

| Bar Size, in. | Transverse Rupture Stress, p. s. i. | Deflection, in. | Tensile Strength, p. s. i. | BHN | Impact Strength, ft.-lb. |
|---------------|-------------------------------------|-----------------|----------------------------|-----|--------------------------|
| 1.6           | 103,600                             | 1.75            | 39,000                     | 158 | -----                    |
| 1.2           | 105,300                             | >2              | 37,400                     | 156 | -----                    |
| 0.875         | 106,100                             | 1.60            | 36,700                     | 172 | 120                      |
| 0.6           | 93,200                              | 0.65            | 35,800                     | 174 | -----                    |

Treated: T. C., 3.03; Si, 3.18; Mn, 5.9; S, 0.018; P, 0.053; Ni, 12.93 Ce, 0.023 per cent

#### EXAMPLE 10

When the nickel content of nodular cast iron exceeds about 10 per cent it is not necessary for the iron to be hypereutectic according to the formula: per cent C/(for eutectic) = 4.3 -  $\frac{1}{3}$  (per cent Si + per cent P). Therefore the treatment can be readily applied to ordinary nickel-containing austenitic irons. In Table 9 the chemical analyses and mechanical properties of treated and untreated nickel-containing iron are given for material cast in the form of 0.875-in. diameter test bars.

Table 9.—Mechanical properties of nickel-containing iron

|                | Composition, per cent |       |       |       |       |       |       |       |       |
|----------------|-----------------------|-------|-------|-------|-------|-------|-------|-------|-------|
|                | T.C.                  | Si    | Mn    | S     | P     | Cr    | Cu    | Ni    | Ce    |
| Untreated..... | 2.76                  | 2.68  | 0.45  | 0.027 | 0.024 | 1.74  | 6.74  | 13.24 | 0.045 |
| Treated.....   | -----                 | ----- | 0.007 | ----- | ----- | ----- | ----- | ----- | ----- |

|                | Transverse Rupture Stress, p. s. i. | Deflection, in. | Tensile Strength, p. s. i. | BHN |
|----------------|-------------------------------------|-----------------|----------------------------|-----|
| Untreated..... | 65,300                              | 0.47            | 27,300                     | 146 |
| Treated.....   | 106,600                             | 0.86            | 46,100                     | 185 |

The structure of the untreated bar is shown in Fig. 30 to consist of undercooled graphite in a matrix of austenite, together with a small amount of carbide. The structure of the treated bar is illustrated in Fig. 31, and is seen to have nodular graphite in a matrix of austenite with rather more carbide than the untreated bar. The treated material was, in this case, produced by treatment of the melt with misch metal alone — the double treatment technique was not employed. It is apparent that the nodular nickel-containing iron has mechanical properties considerably in excess of those in the untreated material.

#### EXAMPLE 11

With relatively high sulphur contents the yield of cerium depends upon the extent of the desulphurization produced by the addition. In such cases, if desulphurization by the cerium is allowed to take place, the yield of cerium will be low, but it is imperative for the success of the process that this desulphurization should occur.

Table 10.—Desulphurizing influence of cerium

|    | Addition of Ce as Misch metal, per cent | S, per cent | Ce (by Analysis), per cent | Structure         |
|----|-----------------------------------------|-------------|----------------------------|-------------------|
| 30 | 0.1                                     | 0.099       | 0.066                      | Flake graphite.   |
|    | 0.2                                     | 0.051       | 0.071                      | Do                |
|    | 0.3                                     | 0.014       | 0.063                      | Nodular graphite. |

If desulphurization by the cerium addition is not effected, the apparent yield of cerium will be high, but this cerium, as found by chemical analysis, will be largely combined with the sulphur and hence will not operate to produce nodular structures. As an instance of the desulphurizing influence of cerium, the figures in Table 10 may be quoted for the treatment of cupola-melted nickel-containing iron. These figures clearly indicate the importance of the cerium not combined with the sulphur in determining the graphite structure.

#### EXAMPLE 12

The production of nodular cast irons by the process described herein presents no special metallurgical difficulties with batch-type melting units if high-carbon and low-sulphur charges are used. The material has been successfully produced in direct- and indirect-arc furnaces, high-frequency induction furnaces, crucible furnaces and oil-fired rotary furnaces by melting low-sulphur (of the order of 0.03 per cent sulphur) hematite pig iron and making the appropriate additions of cerium in the ladle.

With the cupola melting furnace the production of molten iron suitable for the application of this process becomes more difficult and, in general, special precautions need to be taken to ensure that the metal is of the correct composition. The production of high-carbon or hypereutectic cast irons from the cupola is not a difficult matter provided the average carbon content of the charge is reasonably high.

Production of satisfactory low-sulphur contents presents much more difficulty. Even when low-sulphur charges are used there generally is a sulphur pick-up from the coke and the sulphur content of the metal tapped will be too high to allow immediate treatment with misch metal, and it therefore becomes necessary to interpose a preliminary desulphurizing treatment of the metal in the ladle.

If the sulphur content of the metal tapped

from the cupola is within the range of 0.05-0.08 per cent, it is possible to desulphurize the metal to a satisfactory low-sulphur content by one treatment with sodium carbonate, preferably using a ladle lined with basic refractory. With sulphur contents in excess of 0.08 per cent the "double ladle" technique of desulphurizing may have to be applied.

Nodular cast irons can be produced from the cupola, using the sodium carbonate desulphurizer prior to the addition of the misch metal. The mechanical properties given in Table 11 illustrate the results which have been obtained from a cupola operating under industrial conditions.

Table 11. — Mechanical properties of cupola-melted cast iron desulphurized with sodium carbonate

[Composition; T. C., 3.69; Si, 2.77; Mn, 0.63; S, 0.005; P, 0.045; Ce, 0.057 per cent.]

| Test Bar Diameter, in. | Transverse Rupture Stress, p. s. i. | Deflection, in. | Tensile Strength, p. s. i. | BHN |
|------------------------|-------------------------------------|-----------------|----------------------------|-----|
| 3.0                    | 106,000                             | 0.51            | 85,000                     | 241 |
| 2.1                    | 142,700                             | 2.14            | -----                      | --- |
| 1.6                    | 152,000                             | 1.30            | -----                      | --- |
| 1.2                    | 137,500                             | 0.95            | 80,400                     | 218 |
| 0.875                  | 174,300                             | 0.83            | 76,500                     | 244 |
| 0.6                    | 179,500                             | 0.53            | -----                      | --- |

These results were obtained from test bars cast from a cupola run in which the metal was tapped directly onto sodium carbonate placed in the bottom of the ladle, the slag thickened with limestone and skimmed off, and then misch metal and silicon-manganese-zirconium added. The micro-structure of all bars of this set had spherulitic nodular graphite. The structure of the 1.2-in. bar is shown in Fig. 32.

For a casting of any given size, there is a maximum proportion of cerium which must not be exceeded if the formation of white iron is to be avoided. By "section size" is meant the thickness of the casting at its smallest cross-section. In Table 12 below are given the approximate maximum proportions of cerium that are permissible in castings of various sizes, where cerium additions alone are concerned; but it is to be understood that this is illustrative only and that the invention is not limited in its applicability to castings of any particular order of magnitude.

Table 12

| Section Size in Inches           | Maximum Percentage of Cerium for Avoidance of White Iron |
|----------------------------------|----------------------------------------------------------|
| Less than $\frac{1}{4}$          | 0.03                                                     |
| $\frac{1}{4}$ - $\frac{1}{8}$    | 0.05                                                     |
| $\frac{1}{8}$ - $\frac{1}{16}$   | 0.10                                                     |
| $\frac{1}{16}$ - $\frac{1}{32}$  | 0.15                                                     |
| $\frac{1}{32}$ - $\frac{1}{64}$  | 0.20                                                     |
| $\frac{1}{64}$ - $\frac{1}{128}$ | 0.25                                                     |

For any section size the minimum amount of cerium (not combined with sulphur) effective to produce the desired result is, as already indicated hereinabove, 0.015 to 0.02 per cent, that is, on the order of about 0.02 per cent. Addition to the melt of enough cerium to give more than this minimum in the cast metal may assist, however, in ensuring that every part of the casting contains at least the minimum amount of cerium and, as is shown in Example 2, for instance, the addition of more cerium within the prescribed

limits, may materially enhance the improvement in mechanical properties.

Where the described double treatment technique is employed, the cerium content of the novel gray cast irons is no longer limited to the maxima given in Table 12, and the amount required to yield maximum mechanical properties can be employed without risk of producing white iron. Generally speaking, however, about 0.50 per cent cerium (uncombined with sulphur) in the casting can be regarded as the practical maximum, and it is seldom necessary to exceed 0.25 per cent. In the great majority of cases, gray cast irons produced in accordance with the invention and containing not more than about 0.10 per cent cerium are eminently satisfactory.

It may be pointed out that, for accurate determination of small quantities of cerium in cast iron, no reliable analytical methods were available until comparatively recently. In connection with work leading to the present invention, it was therefore necessary to arrange for the development of special analytical procedure (The Analyst, vol. 73, pages 275-282, May 1948). This was employed in obtaining the analytical figures for cerium given herein.

The requirement that cerium-treated cast irons within the scope of the present invention must solidify gray, that is, must be gray when cast, imposes a practical limitation on the amounts of other metals which the untreated cast iron starting material may contain or which may be added thereto. Typical practical maxima are: nickel, 40%; copper, 7%; chromium, 4%; molybdenum, 2%; vanadium, 2%.

The gray cast iron starting material, and also the cerium-treated gray cast iron produced, may contain as little as 0.5 per cent silicon when the deficiency below 2.3 per cent is compensated for by the presence of nickel and/or copper in appropriate amounts on the equivalency basis mentioned hereinabove.

In practicing the new process, the cerium-supplying material, whether it be the element itself or an alloy or compound thereof such as misch metal, is best added to the molten cast iron starting material in the ladle. Certain losses of cerium occur which vary with different operating conditions and for which due allowance must be made in determining the amount of cerium-supplying material to be added. A good procedure is to run the molten iron on to the addition placed, for instance, in the bottom of the ladle.

It is to be understood that all percentages stated herein are by weight.

The cerium-containing nodular gray cast irons of the invention are not ductile and are still relatively brittle. They differ from malleable cast iron additionally in that their carbon and silicon contents are normally appreciably higher. These two elements, as well as pearlite which most as-cast gray irons of the invention contain, tend to reduce ductility and increase brittleness. In the as-cast condition the novel gray cast irons commonly have a shock resistance considerably better than that of ordinary high-duty gray cast iron, and tensile strengths considerably higher than those of either ordinary malleable cast iron or high-duty gray cast iron. Moreover, a high level of mechanical properties can be achieved in nodular gray cast irons at a fairly low level of hardness.

This application is a continuation-in-part of prior applications of this applicant, Ser. No.

## 19

760,118, filed July 10, 1947, now abandoned, and Ser. No. 23,859, filed April 28, 1948, and co-pending herewith. All subject matter contained in said applications not inconsistent with the present disclosure, is to be regarded as included herein by reference.

What is claimed is:

1. Gray cast iron which contains a small proportion of cerium uncombined with sulphur and in which, in its as-cast state, at least the greater part of its graphite content has a nodular microstructure, said iron containing no sulphur in excess of about 0.02 per cent.

2. Gray cast iron which contains a small proportion of cerium uncombined with sulphur and in which, in its as-cast state, at least the greater part of its graphite content has a nodular microstructure, said iron containing no sulphur in excess of about 0.02 per cent, said iron exhibiting by standard strength tests mechanical properties superior to those of comparable gray cast iron not containing cerium.

3. Gray cast iron according to claim 2, the cerium content of which is within the range of about 0.02 to 0.50 per cent.

4. Gray cast iron according to claim 3, the cerium content of which is within the range of about 0.02 to 0.25 per cent.

5. Gray cast iron according to claim 4, the cerium content of which is within the range of about 0.02 to 0.10 per cent.

6. Gray cast iron according to claim 2, which contains from about 0.02 to 0.50 per cent cerium, is of hypereutectic carbon content, and has a nodular graphite structure that is in substantial part spherulitic.

7. Gray cast iron according to claim 6, in which said nodular graphite structure is partly spherulitic and partly quasi-flake, said iron containing at least about 0.02 per cent and not more than 0.25 per cent cerium.

8. Gray cast iron according to claim 2, which contains from about 0.02 to 0.10 per cent cerium and no sulphur in excess of 0.015 per cent, is of hypereutectic carbon content, and has a nodular graphite structure that is substantially wholly spherulitic.

9. Gray cast iron according to claim 2, which contains from about 0.02 to about 0.05 per cent cerium and no sulphur in excess of 0.015 per cent, is of hypereutectic carbon content, and has a nodular graphite structure that is in substantial part quasi-flake.

10. Gray cast iron which, in the as-cast state, has its graphitic carbon content largely in nodular form; said cast iron containing from about 0.02 to 0.50 per cent cerium, from about 2 to 4.4 per cent total carbon, not more than 0.02 per cent sulphur, not more than 0.6 per cent phosphorus, from 0.5 to 7.0 per cent silicon and, when its silicon content is less than 2.3 per cent, another graphitizing agent comprising at least one metal selected from the group consisting of nickel and copper, the total amount of such other graphitizing agent employed being at least three times the deficit of the silicon percentage from 2.3, but the nickel content of said iron never exceeding 40 per cent and the copper content never exceeding 7 per cent.

## 20

11. The process of producing an improved gray cast iron wherein the graphitic carbon is largely in nodular form, which comprises melting an iron which on casting gives a gray cast iron containing not more than 0.6 per cent of phosphorus, and adding to the melt, before casting, an amount of cerium-supplying material which will result in a gray cast iron containing not less than about 0.02 nor more than 0.5 per cent cerium uncombined with sulphur, and not more than 0.02 per cent sulphur.

12. The process according to claim 11, wherein the amount of cerium added to the melt is such as will result in a gray cast iron containing from about 0.02 to 0.25 per cent cerium.

13. The process according to claim 11, wherein the amount of cerium added to the melt is such as will result in a gray cast iron containing from about 0.02 to 0.10 per cent cerium.

14. The process according to claim 11, which further includes adding a graphitizing inoculant to the melt before casting, but not prior to adding the cerium-supplying material.

15. The process according to claim 14, wherein the graphitizing inoculant is selected from the group consisting of ferro-silicon, silicon-manganese-zirconium and calcium silicide.

16. The process of producing improved gray cast iron which comprises providing a melt of low-sulphur gray iron of hypereutectic carbon content which on casting gives a gray cast iron, adding to said melt while its temperature is within the range 1200° to 1600° C. an amount of a cerium-supplying material sufficient to reduce the sulphur content of the metal to below 0.02 per cent and also to provide cerium free to dissolve in said metal in amount equal to at least 0.02 per cent thereof but not exceeding 0.50 per cent and not sufficient to produce white iron, and casting the cerium-treated melt.

17. The process according to claim 16, which further includes adding a graphitizing inoculant to the melt before casting, but not prior to adding the cerium-supplying material.

18. The process of producing improved gray cast iron which comprises providing a melt of low-sulphur gray iron which on casting gives a gray cast iron, and which contains at least one metal from the group consisting of nickel and copper in amount at least sufficient to compensate for any deficiency there may be in silicon content of said iron below 2.3 per cent, adding to said melt while its temperature is within the range 1200° to 1600° C. an amount of a cerium-supplying material sufficient to reduce the sulphur content of the metal to below 0.02 per cent and also to provide cerium free to dissolve in said metal in amount equal to at least 0.02 per cent thereof but not exceeding 0.50 per cent and not sufficient to produce white iron, and casting the cerium-treated melt.

19. The process according to claim 18, which further includes adding a graphitizing inoculant to the melt before casting, but not prior to adding the cerium-supplying material.

HENTON MORROGH.

No references cited.